

Patented July 12, 1927.

1,635,862

# UNITED STATES PATENT OFFICE.

ROBERT QUAIT, JR., OF BROOKLYN, NEW YORK, ASSIGNOR OF ONE-HALF TO JACOB M. EHRLICH, OF NEW YORK, N. Y.

## PHONOGRAPH RECORD AND METHOD OF PRODUCING THE SAME.

No Drawing.

Application filed July 10, 1923. Serial No. 650,738.

This invention relates to pressed sound-records, formed either as discs or otherwise, whose record-grooves are either laterally-undulatory or vertically-undulatory, and 5 their usual depth is not more than, say, approximately three one-thousandths of an inch, although the depth may be somewhat more or less, as desired. Broadly stated, the invention comprises the new thermo-plastic record-material hereinafter set forth, which may be, and preferably is, used as the surface-coating of a suitable core (which latter need not be, and preferably is not, of thermoplastic material); also the new 10 record-tablets or records having an outer coating of said record-material. The invention comprises further a new record-tablet or record, having between the core and said new surface-coating, an intermediate coating, having a higher point of plasticity than the surface-film; and also a tablet or record having, adhering to the outer surface of said new surface-coating, a thin coating of similar composition to said intermediate 15 coating. The invention consists further of the thin and flexible and rollable record-tablet hereinafter described. The invention consists further of the new process of producing such tablets and records; and also 20 of the various features and steps hereinafter set forth in the appended claims.

The invention will be best understood by reference to the ensuing detailed description of a preferred embodiment thereof, applied 25 to discs; but it must be understood that the invention is not limited to the described features with regard to ingredients, steps, and so forth, as hereinafter disclosed.

The core consists preferably of a compacted body or disc of fibrous material, such 30 as pasteboard, cardboard, laminated paper, or even a thin sheet of paper, fabric, or the like. The core may in any desired manner be rendered waterproof or at least sufficiently repellent to the solvents used, as by treating it with a suitable waterproofing preparation, preferably of the type which is applied in the form of a water-base solution. Whatever type of waterproofing has already been 35 or may be applied, the treated core is allowed or caused to dry out thoroughly, as in a vacuum or in an oven, or by resorting to both expedients, until substantially all the moisture (water or solvent) has evaporated, 40 leaving a thoroughly-dry moisture and sol-

vent-repelling core, hereinafter referred to comprehensively as the treated core.

For the intermediate coating (when used), a substantially pure cellulose-ester, such as 45 nitro-cellulose or cellulose-acetate, or a mixture of such esters, is dissolved in a suitable solvent, such as acetone, ethyl-acetate, methyl-acetone, or some mixture of such or similar solvents; the solution is preferably applied to both faces and also the edge of 50 the treated core in any desired manner, as with a brush or roller, or by dipping or spraying; and the applied solution is then allowed or caused (as above indicated) to dry out until the solvent has substantially 55 evaporated. This intermediate coating is not designed to receive the impressions of the pressing-matrix; and may therefore be quite thin, say, approximately only one or two one-thousandths of an inch thick. 60 This coating serves to unite the subsequently-applied surface-coating and the treated core, besides serving certain other advantageous purposes hereinafter set forth.

For the surface-coating, a cellulose-ester, 65 or a mixture of cellulose-esters, containing (or formed from one or more substances containing) camphor-gum or camphor-gum substitute (or some other suitable gum or resin or a mixture thereof, with or without 70 camphor-gum), is dissolved in a suitable solvent (as indicated above); or a pure cellulose-ester may be thus dissolved, and a suitable proportion of gum-content added to the solution. Then a suitable quantity 75 of finely-commminuted rotten-stone, pumice, or other abrasive, is thoroughly mixed into the solution. Preferably this gum-containing ester is thinned with a greater proportion 80 of solvent than is the aforesaid cellulose ester which constitutes the intermediate coating. Accordingly when such less-diluted solution of cellulose-ester is applied (to 85 form the intermediate coating), its solvent is less prone to enter the minute interstices 90 of the core; and, when the intermediate coating has dried out, it retards entry of the (thinner) solution of gum-containing ester applied to form the outer coating. Said 95 gum-containing solution is applied to one or both faces of the prepared core in any desired manner, as already indicated; and the applied solution is then allowed or caused (as above) to dry out until the solvent has substantially evaporated. Appli- 100

cant has not yet verified the fact, but has reason to believe that the solvent of the surface-coating acts to some extent upon the outer particles of the intermediate coating 5 to which it is applied, resulting in a gradual blending of the adjacent particles of the two coatings and a substantially perfect junction of the two coatings themselves. Inasmuch as the matrix-ridges are to be im- 10 pressed into, and retained by, this surface-coating, the latter may be as much as approximately some three to ten one-thous- andths of an inch in thickness, or even thicker or thinner, if desired. To attain the 15 desired thickness, there may be successive applications of this last-named mixture.

The resultant article, comprising the treated core, the intermediate coating with its relatively-higher point of plasticity and 20 the surface-coating with its relatively-lower plastic point, constitutes the completed record-tablet, and is now ready to have record-grooves pressed into either or both of its faces. The temperature resorted to in the 25 pressing-operation should of course be amply sufficient to render the surface-coating sufficiently plastic; but preferably is insufficient to render the intermediate coating plastic. This is what is meant by the en- 30 suing statements that the plastic point of the intermediate coating is higher than, and that of the surface-coating is lower than, the heat employed in the pressing-operation.

As stated, a pure and essentially gum-free 35 cellulose-ester is practically non-thermoplastic. It is the presence of the gum-content which imparts plasticity to the cellulose-ester, the greater the gum-content the lower the plasticity point. If the gum-con- 40 tent be too great, however, an unsatisfactory record-surface is liable to be produced in the first instance; and even a fairly satisfactory record-surface will rapidly deteriorate where too much gum is present. For ex- 45 ample, it has been found that ordinary celluloid contains too great a gum-content to constitute a satisfactory material for forming the thermoplastic outer coating. Therefore, where the present specification and 50 claims state that the solution for forming said outer coating should contain a suitable amount of gum-content, such statement is to be understood as meaning an appreciably smaller proportion of gum-content than present heretofore in ordinary celluloid for record purposes.

Said intermediate coating serves, as stated, to prevent undue loss of the mixture applied to form the surface-coating. Fur- 60 ther, the dry intermediate coating, especially when essentially free from gum-content, does not become plastic within the range of temperatures employed in the well-known pressing-operation, and therefore in 65 this art is practically non-thermoplastic.

Said intermediate coating serves, during the pressing-operation, as a more or less rigid backing for the surface-coating; indeed, where the floor-face of the die or either face of the matrix or of the record-tablet 70 is not a true plane, or where there may be any deviation from true parallelism of said faces, the fibrous core is believed to act more or less as a cushion, while the intermediate coating (or coatings, if 75 there be one on each face of the core) serves as a more rigid backing for the then-plastic surface-coating. At any rate, better impressions are obtained throughout the entire area of the record-zone, where such 80 intermediate coating is present. The intermediate coating further serves to impart additional stability to the tablet as a whole.

If desired, the core may consist of a thin sheet of paper or fabric, and the coatings, 85 particularly the surface-coating, may be somewhat thinner (for receiving shallower grooves) than above indicated; indeed, the surface-coating (and the intermediate coating) may be applied upon only one face of 90 the core. In such case, the records pressed from such tablets are very flexible and pliable, and may even be rolled up for mailing in a tube. The composition of said coating is sufficiently tough yet pliable, and adhere 95 so faithfully, that there is little or no tendency to cracking when rolled; and yet, when unrolled, the disc may resume approximately its normal plane.

If desired, the aforesaid intermediate 100 coating may be dispensed with, and the aforesaid mixture for the surface-coating may be applied directly upon either or both faces of the treated core.

Again, if desired, a thin film of pure cel- 105 lulose-ester (with little or no gum-content) may be applied upon the outer face of said surface-coating; and in this case the completed tablet is subjected, in the pressing-operation, to a temperature not sufficient to 110 render said film fully plastic, the grooves being impressed into the now-plastic gum-containing coating covered by said film, and the film being somewhat stretched to constitute an indented surfacing which adheres 115 securely to the impressed grooves.

When dry, the aforesaid coatings, whether without gum-content, or containing gum and abrasive, are transparent. Therefore such printed matter as titles, illustrations, advertisements, etc., may be imparted to either or both faces of the core, before said coat- 120 ings are applied and the record-grooves im- pressed; and such printed matter will be clearly visible through the coating or coat- 125 ings. But, if desired, some coloring-matter may be added to either or both of the solu- tions.

The broad invention has thus been de- 130 scribed in all its details, but only for the

sake of clearness. Departures may be made from the described features set forth as to materials and steps of procedure, modifications may be resorted to, and parts of the 5 invention used to the exclusion of other parts, without in any case departing from the spirit of the invention, which is defined by the appended claims.

The invention having thus been fully described, what is claimed is:

1. The herein-described method of producing sound-records, which consists of printing upon a core of fibrous material such as cardboard, treating said printed 15 core with a water-soluble waterproofing, drying it out, applying to said dry treated core a solution of pure transparent and essentially gum-free cellulose-ester, drying out the same to constitute a transparent and 20 practically non-thermoplastic intermediate coating, applying to said dry coated core a mixture of an abrasive in a solution of transparent cellulose-ester containing a suitable amount of gum-content, drying out the same 25 to constitute a transparent surface-coating that will become sufficiently plastic under the heat and pressure of the usual pressing-operation, then under heat impressing the ridges of a record-matrix into said surface- 30 coating, and cooling the same to constitute a pressed record with its aforesaid printing still visible. 95
2. The herein-described method of producing sound-records, which consists of treating 35 a core of fibrous material such as cardboard with a water-soluble waterproofing, drying it out, applying to said dry treated core a solution of pure and essentially gum-free cellulose-ester, drying out the same to constitute an intermediate and practically non-thermoplastic coating, applying to said dry coated core a mixture of an abrasive in a solution of cellulose-ester containing a suitable amount of gum-content, drying the 40 same out to constitute a surface-coating that will become sufficiently plastic under the heat and pressure of the usual pressing-operation, then under heat impressing the ridges of a record-matrix into said surface- 45 coating, and cooling the same to constitute a pressed record. 100
3. The herein-described method of producing sound-records, which consists of printing upon a core of fibrous material such as cardboard, treating said printed core with a water-soluble waterproofing, drying it out, applying to said dry core a mixture of an abrasive in a solution of cellulose-ester containing a suitable amount of gum-content, drying out the same to constitute a transparent surface-coating that will become sufficiently plastic under the heat and pressure of the usual pressing-operation, then under heat impressing the ridges of a record-matrix into said surface-coating, and cooling the same to constitute a pressed sound-record with the aforesaid printing still visible. 110
4. The herein-described method of producing sound-records, which consists of treating a core of fibrous material such as 50 cardboard with a water-soluble waterproofing, drying it out, applying to said dry core a mixture of an abrasive in a solution of cellulose-ester, containing a suitable amount of gum-content, drying out the same to constitute a pressed record. 105
5. The herein-described method of producing sound-records, which consists of printing upon a core of fibrous material such as cardboard, waterproofing and drying out the same, applying to said dry treated core a solution of pure and essentially gum-free transparent cellulose-ester, drying out the same to constitute a transparent and practically non-thermoplastic intermediate coating, applying to said dry coated core a mixture of an abrasive in a solution of transparent cellulose-ester containing a suitable amount of gum-content, drying out the same to constitute a transparent surface-coating that will become sufficiently plastic under the heat and pressure of the usual pressing-operation, then under heat impressing the ridges of a record-matrix into said surface-coating, and cooling the same to constitute a pressed sound-record with the aforesaid printing still visible. 115
6. The herein-described method of producing sound-records, which consists of printing upon a core of fibrous material such as cardboard, waterproofing and drying out said printed core, applying to said dry core a mixture of an abrasive in a solution of transparent cellulose-ester containing a suitable amount of gum-content, drying out the same to constitute a transparent surface-coating that will become sufficiently plastic under the heat and pressure of the usual pressing-operation, then under heat impressing the ridges of a record-matrix into said surface-coating, and cooling the same to constitute a pressed sound-record with the aforesaid printing still visible. 120
7. The herein-described method of producing sound-records, which consists of waterproofing and drying out a core of fibrous material such as cardboard, applying to said dry treated core a solution of pure and essentially gum-free cellulose-ester, drying out the same to constitute an intermediate and practically non-thermoplastic coating, applying to said dry coated core a mixture of an abrasive in a solution of cellulose-ester containing a sufficient amount of gum-content, drying out the same to constitute a pressed record. 125

tute a transparent surface-coating that will become sufficiently plastic under the heat and pressure of the usual pressing-operation, and under heat impressing the ridges of a record-matrix into said surface-coating, and cooling the same to constitute a pressed record.

8. The herein-described method of producing sound-records, which consists of 10 waterproofing and drying out a core of fibrous material such as cardboard, applying to said dry core a mixture of an abrasive in a solution of cellulose-ester containing a sufficient amount of gum-content, drying 15 out the same to constitute a surface-coating that will become sufficiently plastic under the heat and pressure of the usual pressing-operation, then under heat impressing the ridges of a record-matrix into said 20 surface-coating, and cooling the same to constitute a pressed record.

9. The herein-described method of producing sound-records, which comprises applying upon the printed surface of a suitable core a transparent and practically non-thermoplastic intermediate coating, thereafter applying upon said coating a transparent surface-coating that will become sufficiently plastic under the heat and pressure 30 of the usual pressing-operation, and finally impressing record-grooves into said outer coating.

10. The herein-described method of producing sound-records, which comprises applying upon the surface of a suitable core an intermediate and essentially gum-free coating, thereafter applying upon said coating a surface-coating that will become sufficiently plastic under the heat and pressure 40 of the usual pressing-operation, and finally impressing record-grooves into said outer coating.

11. The herein-described method of producing record-tablets, which consists of 45 printing upon a core of fibrous material such as cardboard, treating said printed core with a water-soluble waterproofing, drying it out, applying to said dry treated core a solution of pure transparent and essentially 50 gum-free cellulose-ester, drying out the same to constitute a transparent and practically non-thermoplastic intermediate coating of relatively-high melting-point applying to said dry coated core a mixture of an abrasive in 55 a solution of transparent cellulose-ester containing a suitable amount of gum-content, and drying out the same to constitute a transparent surface-coating that will become sufficiently plastic under the heat and pressure 60 of the usual pressing-operation.

12. The herein-described method of producing record-tablets, which consists of treating a core of fibrous material such as cardboard with a water-soluble waterproofing, 65 drying it out, applying to said dry treated

core a solution of pure and essentially gum-free cellulose-ester, drying out the same to constitute an intermediate and practically non-thermoplastic coating, applying to said dry coated core a mixture of an abrasive in 70 a solution of cellulose-ester containing a suitable amount of gum-content, and drying the same out to constitute a surface-coating that will become sufficiently plastic under the heat and pressure of the usual pressing-operation.

13. The herein-described method of producing record-tablets, which consists of printing upon a core of fibrous material such as cardboard, treating said printed core with 80 a water-soluble waterproofing, drying it out, applying to said dry core a mixture of an abrasive in a solution of cellulose-ester containing a suitable amount of gum-content, and drying out the same to constitute a 85 transparent surface-coating that will become sufficiently plastic under the heat and pressure of the usual pressing-operation.

14. The herein-described method of producing record-tablets, which consists of 90 treating a core of fibrous material such as cardboard with a water-soluble waterproofing, drying it out, applying to said dry core a mixture of an abrasive in a solution of cellulose-ester containing a suitable amount of 95 gum-content, and drying out the same to constitute a surface-coating that will become sufficiently plastic under the heat and pressure of the usual pressing-operation.

15. The herein-described method of producing record-tablets, which consists of 100 printing upon a core of fibrous material such as cardboard, waterproofing and drying out the same, applying to said dry treated core a solution of pure transparent and essentially 105 gum-free cellulose-ester, drying out the same to constitute a transparent and practically non-thermoplastic intermediate coating, applying to said dry coated core a mixture of 110 an abrasive in a solution of transparent cellulose-ester containing a suitable amount of gum-content, and drying out the same to constitute a transparent surface-coating that will become sufficiently plastic under the heat and pressure of the usual pressing-operation.

16. The herein-described method of producing record-tablets, which consists of printing upon a core of fibrous material such as cardboard, waterproofing and drying out 115 said printed core, applying to said dry core a mixture of an abrasive in a solution of transparent and essentially gum-free cellulose-ester containing a suitable amount of 120 gum-content and drying out the same to constitute a transparent surface-coating that will become sufficiently plastic under the heat and pressure of the usual pressing-operation.

17. The herein-described method of pro-

ducing record-tablets, which consists of waterproofing and drying out a core of fibrous material such as cardboard, applying to said dry treated core a solution of pure and essentially gum-free cellulose-ester, drying out the same to constitute an intermediate and practically non-thermoplastic coating applying to said dry coated core a mixture of an abrasive in a solution of cellulose-ester containing a suitable amount of gum-content, and drying out the same to constitute a transparent surface-coating having a sufficiently-low melting-point to be rendered plastic under the heat and pressure of the usual pressing-operation.

18. The herein-described method of producing record-tablets, which consists of waterproofing and drying out a core of fibrous material such as cardboard, applying to said dry core a mixture of an abrasive in a solution of cellulose-ester containing a suitable amount of gum-content and drying out the same to constitute a surface-coating having a sufficiently-low melting-point to be rendered plastic under the heat and pressure of the usual pressing-operation.

19. The herein-described method of producing record-tablets, which comprises applying upon the printed surface of a suitable core a transparent and practically non-thermoplastic intermediate coating, and then applying upon said coating a transparent surface-coating having a sufficiently-low melting-point to be rendered plastic under the heat and pressure of the usual pressing-operation.

20. The herein-described method of producing record-tablets, which comprises applying upon the surface of a suitable core an intermediate and practically non-thermoplastic coating, and then applying upon said coating a surface-coating having a sufficiently-low melting-point to be rendered plastic under the heat and pressure of the usual pressing-operation.

21. The herein-described sound-record, comprising a moisture-repellant core of fibrous material which has printing upon its surface, a transparent intermediate coating of essentially gum-free cellulose-ester adhering thereto, and a transparent surface-coating of cellulose-ester adhering thereto and containing abrasive and also a suitable amount of gum-content to render said coating sufficiently plastic under the heat and pressure of the pressing-operation, said surface coating having record-grooves located within the depth thereof, and said printing being visible through said coatings.

22. The herein-described sound-record, comprising a moisture-repellant core of fibrous material which has printing upon its surface, and a transparent surface-coating of essentially gum-free cellulose-ester secured thereto and containing abrasive and also a

suitable amount of gum-content to render said coating sufficiently plastic under the heat and pressure of the usual pressing-operation, said coating having record-grooves located within the depth thereof and with said printing being visible through said coating.

23. The herein-described sound-record, comprising a moisture-repellant core of fibrous material, an intermediate coating of essentially gum-free cellulose-ester adhering thereto, and a surface-coating of cellulose-ester adhering thereto and containing abrasive and also a suitable amount of gum-content to render said coating sufficiently plastic under the heat and pressure of the usual pressing-operation, said outer coating having record-grooves located in the depth thereof.

24. A resilient and rollable record-tablet comprising a suitable core, a resilient and non-thermoplastic intermediate coating, and a resilient and thermoplastic surface-coating suitable to receive and retain record-grooves.

25. The herein-described sound-record, comprising a suitable core which has printing on its surface, a transparent and practically non-thermoplastic intermediate coating, a transparent surface-coating of thermoplastic material having record-grooves located within the depth thereof, said printing being visible through said coatings.

26. The herein-described sound-record, which comprises a suitable core, an intermediate coating of relatively-high melting-point, a surface-coating of relatively-low melting-point, and record-grooves located entirely within the depth of said surface-coating.

27. The herein-described record-tablet, comprising a moisture-repellant core of fibrous material which has printing upon its surface, a transparent intermediate coating of essentially gum-free cellulose-ester adhering thereto, and a transparent surface-coating of cellulose-ester adhering thereto and containing abrasive and also a suitable amount of gum-content to render it sufficiently plastic under the heat and pressure of the pressing-operation.

28. The herein-described record-tablet, comprising a moisture-repellant core of fibrous material which has printing upon its surface, and a transparent surface-coating of cellulose-ester secured thereto and containing abrasive and also sufficient gum to render said coating plastic under the heat and pressure of the usual pressing-operation, said printing being visible through said coating.

29. The herein-described record-tablet, comprising a moisture-repellant core of fibrous material, an intermediate coating of essentially gum-free cellulose-ester adhering thereto, and a surface-coating of cellulose-ester adhering thereto and containing abrasive and also a suitable amount of gum-

content to render said surface coating sufficiently plastic under the heat and pressure of the pressing-operation.

30. A record-tablet comprising a resilient and non-thermoplastic under-coating and a resilient and thermoplastic outer coating which is suitable to receive and retain record-grooves.

31. The herein-described record-tablet, comprising a suitable core which has printing on its surface, a transparent intermediate and practically non-thermoplastic coating of relatively-high melting-point, and a transparent and sufficiently thermoplastic surface-coating of relatively-low melting point.

32. The herein-described record-tablet, comprising a suitable core, an intermediate coating containing an essentially gum-free cellulose-ester, and a surface-coating containing cellulose-ester having a proportion of gum-content appreciably lower than that of ordinary celluloid.

33. A thin flexible record-disc consisting of a core having a coating of practically pure

and gum-free cellulose-ester and another 25 coating of cellulose-ester containing gum and abrasive, the last-named coating being suitable to receive and retain record-grooves, and said disc being sufficiently pliable and resilient to be rolled up and to retain its shape 30 when unrolled.

34. A record-tablet having a transparent under-coating of practically pure and gum-free cellulose-ester, a transparent outer coating of cellulose-ester containing gum and abrasive, and a transparent outside film of the first-named ester, said outer coating and film being suitable to receive and retain record-grooves.

35. A record-tablet having an under coating of practically pure and gum-free cellulose-ester, an outer coating of cellulose-ester containing gum and abrasive, and an outside film of the first-named ester, said outer coating and film being suitable to receive and retain record-grooves.

ROBERT QUAIT, JR.